

# United States Patent Office

3,329,619

Patented July 4, 1967

1

3,329,619

## PICKLING FERROUS METAL

Robert M. Hudson, Churchill Borough, and Clair J. Warning, Plum Borough, Pa., assignors to United States Steel Corporation, a corporation of Delaware  
No Drawing. Filed Aug. 2, 1965, Ser. No. 476,708  
4 Claims. (Cl. 252—148)

This invention relates to pickling. More particularly, the invention is directed to a pickling composition and to a method of pickling ferrous metal. The term "ferrous metal" as used herein refers to iron, iron alloys and steel. 10

To prepare ferrous metal sheet, strip, etc. for subsequent processing, it is frequently desirable to remove

$$I = 100 \left[ \frac{(\text{Sample's weight change, in uninhibited acid}) - (\text{Sample's weight change, with inhibitor})}{(\text{Sample's weight change in uninhibited acid})} \right]$$

$$L = 100 \left[ \frac{(\text{Sample's hydrogen concentration, uninhibited acid}) - (\text{Sample's hydrogen concentration, with inhibitor})}{(\text{Sample's hydrogen concentration, uninhibited acid})} \right]$$

oxide coating, formed during manufacturing, from the surface. The presence of oxide coating, referred to as "scale" is objectionable when the material is to undergo subsequent processing. Thus, for example, oxide scale must be removed and a clean surface provided if satisfactory results are to be obtained from hot rolled sheet and strip in any operation involving deformation of the product. Similarly, steel prepared for drawing must possess a clean surface and removal of the oxide scale therefrom is essential since the scale tends to shorten drawing-die life as well as destroy the surface smoothness of the finished product. Oxide removal from sheet or strip is also necessary prior to coating operations to permit proper alloying or adherence of the coating to the ferrous metal strip or sheet. Prior to cold reduction, it is necessary that the oxide formed during hot rolling be completely removed to preclude surface irregularities and enable uniform reduction of the work.

The chemical process used to remove oxide from metal surfaces is referred to as "pickling." Typical pickling processes involve the use of aqueous acid solutions, usually inorganic acids, into which the metal article is immersed. The acid solution reacts with the oxides to form hydrogen and a salt of the acid. A common problem in this process is "overpickling" which is a condition resulting when the ferrous metal remains in the pickling solution after the oxide scale is removed from the surface and the pickling solution reacts with the ferrous metal base. An additional difficulty in pickling results from the liberated hydrogen being absorbed by the metal base and causing hydrogen embrittlement. To overcome the aforementioned problems in pickling, it has been customary to add inhibitors to the pickling solution. Although most inhibitors in present use are effective in preventing of overpickling, many do not prevent hydrogen absorption and consequent hydrogen embrittlement. A number of known inhibitors such as some organic compounds containing sulfur have been found to actually promote hydrogen embrittlement.

The present invention avoids the above-described problems in pickling ferrous metal articles and provides a pickling composition which minimizes both overpickling and hydrogen embrittlement. Thus the pickling inhibitors described herein not only prevent excessive dissolution of the ferrous metal base but effectively limit the amount of hydrogen absorption thereby during pickling. According to the invention, a pickling composition for ferrous metal is provided which comprises a pickling acid such as sulfuric or hydrochloric acid and a small but effective amount of a pyrrole ring compound from the group consisting of pyrrole, pyrrolidine, 1-methylpyrrole, 2,5-dimethylpyrrole, indole, indoline, and 2-methylindole, 2,5-dimethylindole or 3-pyrrolidine to inhibit both metal dissolution and hydrogen embrittlement. Ferrous metal articles are pickled

2

by contacting the surface (usually by immersion in the pickling solution) with a pickling composition as described to remove oxide from their surface with minimum dissolution and hydrogen embrittlement thereof and then washing the ferrous metal to remove the pickling composition therefrom.

The effectiveness of pickling inhibitors is measured by the ability to minimize dissolution of the metal base (in overpickling) and to limit hydrogen absorption. The following relationships have been devised as a means of measuring relative effectiveness of inhibitors in both of these categories. These relationships are as follows:

20 The above equations give an indication of the percent inhibition (I) and percent limitation of hydrogen absorption (L). The sample's weight change in the uninhibited acid refers to the change in the sample's weight due to dissolution by the acid. The sample's weight change with the inhibitor refers to change in weight of the sample in an acid solution containing the specified pickling inhibitor. All measurements are made after lapse of the same time period and in the data provided herein a standard 4-hour period was used. In the second equation, the "sample's hydrogen concentration, uninhibited acid" refers to the amount of hydrogen that is driven off by warm extraction of the sample, i.e. heating at 160-165° C. for 16 hours. The value used in this equation is in "cc. of hydrogen/100 grams sample." Similarly the "sample's hydrogen concentration, with inhibitor" refers to the amount of hydrogen obtained in the same manner (i.e. by "warm extraction") from the sample contacted with pickling acid composition containing a specified pickling inhibitor; also in both these cases for the same unit time, e.g. 4 hours.

30 40 45 50 If no weight loss occurs when a specimen is immersed in an inhibited acid then  $I=100$ , which is the maximum inhibitor effectiveness possible for a given acid-immersion and time combination. Similarly, if no hydrogen is absorbed by specimens immersed for a unit time in an inhibited acid, then  $L=100$ . Often an inhibitor will be effective for limiting weight loss during pickling but less effective or completely ineffective for preventing hydrogen absorption by the ferrous metal samples. For an inhibitor that increases weight loss I is negative and for one that increases hydrogen absorption L is negative.

55 The results of a number of tests of various pickling inhibitors including those within the purview of the invention are presented in Tables I and II below. The samples used were of commercially available normalized and temper-rolled low-carbon sheet steel of the following composition: 0.022% carbon, 0.14% manganese, 0.007% phosphorus, 0.017% sulfur, 0.004% silicon, 0.015% copper, <0.002% nickel, 0.010% chromium, <0.002% aluminum, the balance being essentially iron. 60 The samples were 2 x 3/8" and 0.036" thick and were vapor degreased with trichloroethylene before use. All the samples were pickled at 100° F. for 4 hours by immersion in 2 N hydrochloric acid solution with and without inhibitors (Table I) or 2 N sulfuric acid solution with and without inhibitors (Table II). The samples were weighed prior to pickling and, in the case of the hydrogen absorption test, after extraction of the hydrogen absorbed during pickling. The hydrogen concentration in the pickled steel specimens was determined by warm extraction according to the method described by R. M. Hudson et al., Journal American Ceramic Society, 41, 23 (1958).

65 70 75 Tables I and II below indicate the relative effectiveness

of inhibitors present in different concentrations. For some, increasing the quantity of inhibitors does not provide a proportional increase in effectiveness, for others increasing the amount of inhibitors increases their effectiveness.

Thus for some materials I values significantly increased with an increase in concentration, whereas the effectiveness of the better inhibitors does not depend greatly on concentration.

TABLE I.—EFFECTIVENESS OF INHIBITORS FOR PICKLING OF LOW-CARBON STEEL IN 2 N HYDROCHLORIC ACID SOLUTIONS AT 100° F. (4-HOUR IMMERSION)

| Compound            | Concentration Used, percent | Inhibition                            |                       | Hydrogen Absorption               |                                              |
|---------------------|-----------------------------|---------------------------------------|-----------------------|-----------------------------------|----------------------------------------------|
|                     |                             | Weight Loss, mg. per cm. <sup>2</sup> | Percent Inhibition, I | Hydrogen Absorbed, cc. per 100 g. | Percent Limitation of Hydrogen Absorption, L |
| Pyrrole             | 0.05 Vol.                   | 0.3                                   | 93                    | 0.7                               | 84                                           |
| Do                  | 0.1 Vol.                    | 0.3                                   | 91                    | 0.6                               | 87                                           |
| Do                  | 0.2 Vol.                    | 0.2                                   | 94                    | 0.8                               | 82                                           |
| 3-Pyrroline         | 0.05 Vol.                   | 1.1                                   | 68                    | 2.3                               | 48                                           |
| Do                  | 0.1 Vol.                    | 1.4                                   | 61                    | 2.3                               | 49                                           |
| Do                  | 0.2 Vol.                    | 0.6                                   | 84                    | 1.2                               | 74                                           |
| Pyrrolidine         | 0.05 Vol.                   | 1.6                                   | 54                    | 3.1                               | 30                                           |
| Do                  | 0.1 Vol.                    | 1.5                                   | 57                    | 2.6                               | 42                                           |
| Do                  | 0.2 Vol.                    | 1.2                                   | 67                    | 2.1                               | 53                                           |
| 1-Methylpyrrole     | 0.05 Vol.                   | 0.2                                   | 93                    | 0.4                               | 91                                           |
| Do                  | 0.1 Vol.                    | 0.4                                   | 89                    | 0.8                               | 82                                           |
| Do                  | 0.2 Vol.                    | 0.1                                   | 96                    | 0.2                               | 96                                           |
| 2,5-Dimethylpyrrole | 0.05 Vol.                   | 0.3                                   | 91                    | 0.9                               | 81                                           |
| Do                  | 0.1 Vol.                    | 0.3                                   | 91                    | 0.6                               | 87                                           |
| Do                  | 0.2 Vol.                    | 0.2                                   | 93                    | 0.5                               | 89                                           |
| Indole              | 0.05 Wt.                    | 0.1                                   | 97                    | 0.1                               | 98                                           |
| Do                  | 0.1 Wt.                     | 0.1                                   | 97                    | 0.3                               | 93                                           |
| Do                  | 0.2 Wt.                     | 0.03                                  | 99                    | 0.1                               | 97                                           |
| Indoline            | 0.05 Vol.                   | 0.9                                   | 74                    | 2.5                               | 45                                           |
| Do                  | 0.1 Vol.                    | 0.3                                   | 91                    | 0.6                               | 87                                           |
| Do                  | 0.2 Vol.                    | 0.5                                   | 87                    | 1.1                               | 76                                           |
| 2-Methylindole      | 0.05 Wt.                    | 0.7                                   | 81                    | 1.6                               | 64                                           |
| Do                  | 0.1 Wt.                     | 0.7                                   | 80                    | 1.3                               | 71                                           |
| Do                  | 0.2 Wt.                     | 0.2                                   | 95                    | 0.4                               | 91                                           |
| 3-Methylindole      | 0.05 Wt.                    | (1)                                   | 14                    | 4.3                               | 4                                            |
| Do                  | 0.1 Wt.                     |                                       |                       |                                   |                                              |
| Do                  | 0.2 Wt.                     |                                       |                       |                                   |                                              |
| 2,5-Dimethylindole  | 0.05 Wt.                    | 1.1                                   | 69                    | 2.3                               | 48                                           |
| Do                  | 0.1 Wt.                     | 1.2                                   | 66                    | 2.5                               | 44                                           |
| Do                  | 0.2 Wt.                     | 0.6                                   | 82                    | 1.7                               | 63                                           |
| Carbazole           | 0.05 Wt.                    | (1)                                   | 11                    | 4.4                               | 2                                            |
| Do                  | 0.1 Wt.                     |                                       |                       |                                   |                                              |
| Do                  | 0.2 Wt.                     |                                       |                       |                                   |                                              |
| Uninhibited         |                             | 3.5                                   | 0                     | 4.5                               | 0                                            |

<sup>1</sup> Not tested.

TABLE II.—EFFECTIVENESS OF INHIBITORS FOR PICKLING OF LOW-CARBON STEEL IN 2 N SULFURIC ACID SOLUTIONS AT 100° F. (4-HOUR IMMERSION)

| Compound            | Concentration Used, percent | Inhibition                            |                       | Hydrogen Absorption               |                                              |
|---------------------|-----------------------------|---------------------------------------|-----------------------|-----------------------------------|----------------------------------------------|
|                     |                             | Weight Loss, mg. per cm. <sup>2</sup> | Percent Inhibition, I | Hydrogen Absorbed, cc. per 100 g. | Percent Limitation of Hydrogen Absorption, L |
| Pyrrole             | 0.05 Vol.                   | 0.8                                   | 89                    | 1.6                               | 77                                           |
| Do                  | 0.1 Vol.                    | 0.9                                   | 88                    | 0.9                               | 87                                           |
| Do                  | 0.2 Vol.                    | 0.7                                   | 91                    | 1.4                               | 79                                           |
| 3-Pyrroline         | 0.05 Vol.                   | (1)                                   | 20                    | 6.8                               | 0                                            |
| Do                  | 0.1 Vol.                    |                                       |                       |                                   |                                              |
| Do                  | 0.2 Vol.                    |                                       |                       |                                   |                                              |
| Pyrrolidine         | 0.05 Vol.                   | 4.9                                   | 36                    | 6.7                               | 1                                            |
| Do                  | 0.1 Vol.                    | 4.5                                   | 41                    | 5.8                               | 15                                           |
| Do                  | 0.2 Vol.                    | 3.6                                   | 53                    | 5.6                               | 18                                           |
| 1-Methylpyrrole     | 0.05 Vol.                   | 0.9                                   | 89                    | 1.0                               | 85                                           |
| Do                  | 0.1 Vol.                    | 1.1                                   | 86                    | 1.4                               | 79                                           |
| Do                  | 0.2 Vol.                    | 0.6                                   | 92                    | 1.6                               | 77                                           |
| 2,5-Dimethylpyrrole | 0.05 Vol.                   | 1.5                                   | 80                    | 2.4                               | 65                                           |
| Do                  | 0.1 Vol.                    | 1.5                                   | 80                    | 2.4                               | 65                                           |
| Do                  | 0.2 Vol.                    | 1.1                                   | 86                    | 1.6                               | 76                                           |
| Indole              | 0.05 Wt.                    | 1.6                                   | 79                    | 2.5                               | 64                                           |
| Do                  | 0.1 Wt.                     | 0.2                                   | 97                    | 0.7                               | 90                                           |
| Do                  | 0.2 Wt.                     | 0.2                                   | 97                    | 0.9                               | 87                                           |
| Indoline            | 0.05 Vol.                   | 3.0                                   | 61                    | 4.4                               | 36                                           |
| Do                  | 0.1 Vol.                    | 1.2                                   | 84                    | 1.3                               | 81                                           |
| Do                  | 0.2 Vol.                    | 1.0                                   | 87                    | 1.4                               | 80                                           |
| 2-Methylindole      | 0.05 Wt.                    | 2.9                                   | 61                    | 4.8                               | 30                                           |
| Do                  | 0.1 Wt.                     | 4.2                                   | 45                    | 4.2                               | 38                                           |
| Do                  | 0.2 Wt.                     | 1.6                                   | 78                    | 1.6                               | 76                                           |
| 3-Methylindole      | 0.05 Wt.                    | (1)                                   | 8                     | 6.6                               | 3                                            |
| Do                  | 0.1 Wt.                     |                                       |                       |                                   |                                              |
| Do                  | 0.2 Wt.                     |                                       |                       |                                   |                                              |
| 2,5-Dimethylindole  | 0.05 Wt.                    | (1)                                   | 12                    | 6.4                               | 6                                            |
| Do                  | 0.1 Wt.                     |                                       |                       |                                   |                                              |
| Do                  | 0.2 Wt.                     |                                       |                       |                                   |                                              |
| Carbazole           | 0.05 Wt.                    | (1)                                   | -1                    | 8.5                               | -25                                          |
| Do                  | 0.1 Wt.                     |                                       |                       |                                   |                                              |
| Do                  | 0.2 Wt.                     |                                       |                       |                                   |                                              |
| Uninhibited         |                             | 7.6                                   | 0                     | 6.8                               | 0                                            |

<sup>1</sup> Not tested.

As can be seen, pickling inhibitors differ greatly in their effectiveness, that is, the I and L values associated with the inhibitor. Moreover, the data illustrate the unpredictability of inhibitor effectiveness since, as shown, some pyrrole ring compounds would not be commercially useful while others are.

If maximum protection against overpickling is desired for a given application, the inhibitors exhibiting I values of 80 or above may be preferred. For many applications, however, the residence time of steel in the pickling bath is relatively short and inhibitors exhibiting lower I values, e.g.  $I=40$  may be considered useful. In a typical commercial practice, inhibitor concentration on the order of 0.1 volume or weight percent in acid solution would be used. As shown in Tables I and II, many inhibitors can be used at 0.05 volume or weight percent. It is generally desirable to use the least amount of inhibitor which provides the desired results.

It is also known that many materials which are effective in limiting metal dissolution are relatively ineffective in limiting hydrogen absorption, thus there are many instances where high I values are coupled with low or poor L values. Inhibitors having minimum L values of from 40 to 50 are acceptable for many applications. For applications in which hydrogen absorbed during pickling would not have an opportunity to escape before subsequent processing, the need for high L value would be greater than for situations where the time lapse following the pickling operation is longer. Thus where steel strips are electrolytically coated immediately after pickling and rinsing, the time lag is slight and pickling inhibitors having relatively high L values should be used.

The quantity of inhibitors used is related to the pickling acid strength. For example, if 0.1 volume or weight percent inhibitor concentration is effective for a 2 N acid solution, then 0.05 volume or weight percent inhibitor concentration should be adequate for 1 N acid solution. In the same way, 0.2 volume or weight percent inhibitor should be adequate for a 4 N acid solution.

We claim:

1. A pickling composition for ferrous metal consisting essentially of a pickling acid from the group consisting of sulfuric acid and hydrochloric acid and a small but

effective amount of a pyrrole ring compound from the group consisting of pyrrole, pyrrolidine, 1-methylpyrrole, 2,5-dimethylpyrrole, indole, indoline, and 2-methylindole, 2,5-dimethylindole and 3-pyrroline to inhibit both dissolution and hydrogen embrittlement of said ferrous metal by said pickling acid.

2. A pickling composition according to claim 1 wherein in said pickling acid is sulfuric and said pyrrole ring compound is a member from the group consisting of pyrrole, pyrrolidine, 1-methylpyrrole, 2,5-dimethylpyrrole, indole, indoline and 2-methylindole.

3. A method of pickling a ferrous metal surface comprising contacting said surface with a composition comprising a pickling acid from the group consisting of sulfuric acid and hydrochloric acid and a pyrrole ring compound from the group consisting of pyrrole, pyrrolidine, 1-methylpyrrole, 2,5-dimethylpyrrole, indole, indoline, and 2-methylindole, 2,5-dimethylindole and 3-pyrroline, said pickling composition being effective to remove oxides from said ferrous metal surface with minimum dissolution and hydrogen embrittlement thereof, and washing said ferrous metal to remove said pickling composition.

4. A method according to claim 3 wherein said pickling acid is sulfuric acid and said pyrrole ring compound is a member from the group consisting of pyrrole, pyrrolidine, 1-methylpyrrole, 2,5-dimethylpyrrole, indole, indoline and 2-methylindole.

#### References Cited

##### UNITED STATES PATENTS

|           |         |             |       |           |
|-----------|---------|-------------|-------|-----------|
| 1,719,650 | 7/1929  | Chamberlain | ----- | 252—390   |
| 1,746,679 | 2/1930  | Rhodes      | ----- | 252—390   |
| 2,043,257 | 6/1936  | Missback    | ----- | 252—390 X |
| 3,056,746 | 10/1962 | Brightly    | ----- | 252—148   |
| 3,214,433 | 10/1965 | Hester      | ----- | 252—390 X |

##### FOREIGN PATENTS

|         |        |                |
|---------|--------|----------------|
| 765,522 | 1/1957 | Great Britain. |
|---------|--------|----------------|

40 LEON D. ROSDOL, *Primary Examiner.*

SAMUEL H. BLECH, JOHN T. FEDIGAN,  
*Assistant Examiners.*